

1

3,288,576  
TREATING COAL

Emile D. Pierron, Creve Coeur, and Philip E. McIntyre,  
Des Peres, Mo., assignors to Monsanto Company, a 5  
corporation of Delaware  
No Drawing. Filed Sept. 3, 1963, Ser. No. 306,326  
8 Claims. (Cl. 44—1)

This invention relates to a method of treating coal and to coal compositions resistant to degradation.

Coal is susceptible to oxidation. The grinding of coal, required for certain uses, accelerates the oxidation by exposing new surfaces. Oxidation of coal is undesirable for several reasons. For example, coal storage piles have been destroyed because of spontaneous combustion; the slow oxidation under conditions that do not permit dissipation of the heat evolved results in increase in temperature, acceleration of oxidation processes, accumulation of more heat until active combustion starts. Another costly effect of coal oxidation is the loss of heating value during storage of reserve fuel pile at power plants. In the case of high volatile matter bituminous C or coal of lower rank, loss in B.t.u. values during storage could amount to 5 to 10% of the original heating value of the coal. The stock of coking coal at a metallurgical coke plant may deteriorate to the point that no satisfactory coke can be produced.

Although it has been proposed to protect coal by coating of the surface thereof so as to present impervious physical barrier between it and the atmosphere, these treatments have either been ineffective or uneconomical. It has now been found that phosphite esters inhibit the oxidation of coal. The phosphite ester may advantageously be used in combination with a dihydrotrialkylquinoline. The antioxidant will normally be within the range of 250-2,500 parts per million parts of coal. Where the antioxidant is composed of the aforesaid mixture the phosphite ester should be at least 50% and preferably 85% of the total. Thus, the antioxidant composition will be composed of 50-85% phosphite ester and 15-50% dihydrotrialkylquinoline.

As an example of the invention, a high volatile bituminous C rank coal ground to pass a 40 mesh sieve is treated with 750 parts per million of antioxidant. This antioxidant is applied to the ground coal in acetone or methanol solution and the coal so treated is dried at room temperature for a few hours to remove the solvent. The course of the degradation is followed by measuring the oxygen absorption as a function of time. An untreated sample is run as a control. The oxygen absorption is conveniently determined by placing samples of the control and treated material in air-tight containers attached to glass burettes filled with oxygen and measuring the amount of oxygen absorbed. The rate of oxygen uptake for treated samples is significantly lower than for the untreated sample. The effect of oxidation is followed by periodic determination of the heating values. Certain high volatile bituminous B used for metallurgical coke manufacture are usually utilized in coke ovens within a few weeks after mining due to their loss in maximum fluidity produced by oxidation. Maximum fluidity values of the Gieseler plasticity test obtained periodically on untreated and treated samples show that the effect of oxidation can be appreciably minimized, especially within the first 4 weeks after mining.

Examples of the antioxidant compositions comprise

- A. 1 part 6-dodecyl-1,2-dihydro-2,2,4-trimethylquinoline  
5 parts triphenylphosphite
- B. 1 part 6-dodecyl-1,2-dihydro-2,2,4-trimethylquinoline  
5 parts tri(nonylphenyl)phosphite

2

C. 1 part 6-ethoxy-1,2-dihydro-2,2,4-trimethylquinoline  
5 parts tri(nonylphenyl)phosphite

D. Tri(nonylphenyl)phosphite

Compositions A, B and C are applied at a dosage of 750 parts per million parts of coal and Composition D at 625 parts per million parts of coal.

The antioxidants are advantageously applied in either emulsion or solution form. The antioxidant may be dissolved in an organic solvent as described or dispersed as an aqueous medium and the composition applied to coal in any suitable manner. Addition of small amounts of a surface active agent facilitates dispersion. It is now customary to wash coal as it comes from the mine. The antioxidant is advantageously applied through adaptation of equipment already installed for washing coal.

A large number of phosphite esters are available and any of these may be employed in carrying out the method of the present invention. Examples comprise

- 20 Triphenylphosphite  
Tri-o-tolylphosphite  
Tri-m-tolylphosphite  
Tri-p-tolylphosphite  
Trixenyl phosphite  
25 Tri-beta-naphthyl phosphite  
Tri-alpha-naphthyl phosphite  
Tri-p-isopropylphenyl phosphite  
Tri-p-tert. butylphenyl phosphite  
Tri-p-tert. amylphenyl phosphite  
30 Tri-p-phenoxyphenyl phosphite  
Tri-p-benzoyloxyphenyl phosphite  
Tri-p-chlorophenyl phosphite  
Tri-(4-methyl 2,6-di-tert. butylphenyl) phosphite  
Tri-(3-methyl 4,6-di-tert. butylphenyl) phosphite  
35 Tri-(3-dimethylphenyl) phosphite  
Tri-(2,4-dimethylphenyl) phosphite  
Tri-(3,4-dimethylphenyl) phosphite  
Tri-(2,5-dimethylphenyl) phosphite  
Tri-(2,4,6-tri-tert. butylphenyl) phosphite  
40 Tri-(2-methyl 4,6-di-tert. butylphenyl) phosphite  
Tri-(o-octylphenyl) phosphite  
Tri-(p-nonylphenyl) phosphite  
Tri-(p-decylphenyl) phosphite  
Tri-(p-undecylphenyl) phosphite  
45 Tri-(p-dodecylphenyl) phosphite  
Tri-(p-tridecylphenyl) phosphite  
Tri-(p-tetradecylphenyl) phosphite  
Tri-(p-pentadecylphenyl) phosphite  
Tri-(p-hexadecylphenyl) phosphite  
Tri-(p-heptadecylphenyl) phosphite  
50 Tri-(p-octadecylphenyl) phosphite  
Tri-(p-eicosyl-phenyl) phosphite  
Tri-(2-ethylhexylphenyl) phosphite  
p-Octyl-phenyl di(p-nonylphenyl) phosphite  
55 p-Nonyl-phenyl di(p-octyl-phenyl) phosphite  
p-Dodecyl-phenyl di(p-octyl-phenyl) phosphite  
Tris(di-octyl-phenyl) phosphite  
Tris(di-nonyl-phenyl) phosphite  
Tris(p-octyl-phenyl) phosphite  
60 Tri(nonyl-phenyl) phosphite  
Mono octyl-phenyl di(nonyl-phenyl) phosphite  
Mono(nonyl-phenyl) di(octyl-phenyl) phosphite  
Tri(dodecyl-phenyl) phosphite  
Tri(di-nonyl-phenyl) phosphite  
65 Tri(p-tert. amyl-phenyl) phosphite  
Tri(p-octyl-phenyl) phosphite  
Mono(o-sec. amyl phenyl) phosphite  
Mono(p-1,1,3,3-tetramethyl butyl phenyl) phosphite  
Mono(2,4-di-sec. amyl phenyl) phosphite  
70 Mono(2-tert.butyl-5-methyl phenyl) phosphite  
Mono(2,4-di-tert. butyl-5-methyl phenyl) phosphite  
Mono(nonyl phenyl) phosphite

Mono(dodecyl phenyl) phosphite  
 Mono(di-nonyl phenyl) phosphite  
 Mono(p-tert. amyl phenyl) phosphite  
 Mono(n-hexyl phenyl) phosphite  
 Mono(n-heptyl phenyl) phosphite  
 Mono(p-n-decyl phenyl) phosphite  
 Mono(p-n-pentadecyl phenyl) phosphite  
 Mono(p-n-hexadecyl phenyl) phosphite  
 Mono(p-n-octadecyl phenyl) phosphite  
 Mono(alkylaryl) phosphite  
 Mono(di-sec. amyl phenyl) phosphite  
 Mono(2-tert. butyl 4-methyl phenyl) phosphite  
 Mono(phenyl) phosphite  
 Mono(di-tert. butyl m-cresyl) phosphite  
 Ethylene phenyl phosphite  
 Ethylene 2-chlorophenyl phosphite  
 Ethylene 3-chlorophenyl phosphite  
 Ethylene 4-chlorophenyl phosphite  
 Ethylene 2-methylphenyl phosphite  
 Ethylene 3-methylphenyl phosphite  
 Ethylene 4-methylphenyl phosphite  
 Ethylene 4-ethylphenyl phosphite  
 Ethylene 2-cyclohexylphenyl phosphite  
 Ethylene 4-octylphenyl phosphite  
 Ethylene 3-isobutylphenyl phosphite  
 Ethylene 2-dodecylphenyl phosphite  
 Ethylene 4-ethoxyphenyl phosphite  
 Ethylene 4-octyloxyphenyl phosphite  
 2-ethylhexyl bis(p-octylphenyl) phosphite  
 2-ethylhexyl diphenyl phosphite  
 Bis(2-ethylhexyl) phenyl phosphite  
 Bis(2-ethylhexyl) o-tolyl phosphite  
 Bis(2-ethylhexyl) p-tolyl phosphite  
 Bis(2-ethylhexyl) p-octylphenyl phosphite  
 Allyl di-o-tolyl phosphite  
 Allyl bis(p-nonylphenyl) phosphite  
 3-cyclohexen-1-ylmethyl di-o-tolyl phosphite  
 Di-(dodecyl) mono(nonylphenyl) phosphite  
 Di-(octyl) mono(octyl phenyl) phosphite  
 Di-(decyl) mono(nonylphenyl) phosphite  
 Di-(nonyl) mono(decyl phenyl) phosphite  
 Di-(nonyl) mono(dodecyl phenyl) phosphite  
 Di-(2-octyl) mono(nonyl phenyl) phosphite  
 Di-(nonyl) mono(nonyl phenyl) phosphite  
 Di-(undecyl) mono(nonyl phenyl) phosphite  
 Di-(nonyl) mono(octyl phenyl) phosphite  
 Di-(nonyl) mono(undecyl phenyl) phosphite

Similarly, the dihydroquinoline antioxidants are well known and suitable preservatives may be selected therefrom. Although the quinolines are preferably used in conjunction with phosphite esters they may be employed neat for preservation of coal. Examples of suitable quinoline antioxidants comprise 2,2,4-triethyl-1,2-dihydro-6-aralkyl substituted quinolines, as for example 2,2,4-trimethyl-1,2-dihydro-6-aralkylquinolines wherein the aralkyl is benzyl, 1-benzyl-2-phenethyl, 1-phenyl-isopropyl or 1-p-tolyl-isopropyl. Still further examples are

2,2,4-trimethyl-1,2-dihydroquinoline  
 polymeric 2,2,4-trimethyl-1,2-dihydroquinoline  
 2-methyl-2,4-diethyl-1,2-dihydroquinoline  
 2-methyl-2,4-diisopropyl-1,2-dihydroquinoline  
 5 6-methoxy-1,2-dihydro-2,2,4-trimethylquinoline  
 6-ethoxy-1,2-dihydro-2,2,4-trimethylquinoline  
 6-propoxy-1,2-dihydro-2,2,4-trimethylquinoline  
 6-isopropoxy-1,2-dihydro-2,2,4-trimethylquinoline  
 6-butoxy-1,2-dihydro-2,2,4-trimethylquinoline  
 10 6-hexoxy-1,2-dihydro-2,2,4-trimethylquinoline  
 6-phenoxy-1,2-dihydro-2,2,4-trimethylquinoline  
 6-butoxyethoxy-1,2-dihydro-2,2,4-trimethylquinoline  
 6-methoxyethoxy-1,2-dihydro-2,2,4-trimethylquinoline  
 6-diethylamino-1,2-dihydro-2,2,4-trimethylquinoline  
 15 6-butyl-1,2-dihydro-2,2,4-trimethylquinoline and  
 6-phenyl-1,2-dihydro-2,2,4-trimethylquinoline

It is intended to cover all changes and modifications of the examples of the invention herein chosen for purposes of disclosure which do not constitute departures 20 from the spirit and scope of the invention.

What is claimed is:

1. A composition comprising coal having admixed therewith a small amount sufficient to inhibit oxidation of a phosphite ester antioxidant and a 1,2-dihydroquinoline antioxidant.
2. A composition comprising coal having admixed therewith a small amount sufficient to inhibit oxidation of a phosphite ester antioxidant.
3. A composition comprising coal having admixed therewith a small amount sufficient to inhibit oxidation of tri(alkylphenyl) phosphite antioxidant.
4. A composition comprising coal admixed with a small amount sufficient to inhibit oxidation of tri(nonyl phenyl) phosphite.
- 35 5. A composition comprising coal admixed with a small amount sufficient to inhibit oxidation of a tri(nonyl phenyl) phosphite and 6-dodecyl-1,2-dihydro-2,2,4-trimethylquinoline.
6. A composition comprising coal admixed with a small amount sufficient to inhibit oxidation of a dihydroquinoline antioxidant.
7. A composition comprising coal admixed with a small amount sufficient to inhibit oxidation of 6-alkoxy-1,2-dihydro-2,2,4-trimethylquinoline.
- 45 8. A composition comprising coal admixed with a small amount sufficient to inhibit oxidation of 6-alkyl-1,2-dihydro-2,2,4-trimethylquinoline.

#### References Cited by the Examiner

#### UNITED STATES PATENTS

|           |         |                |       |           |
|-----------|---------|----------------|-------|-----------|
| 2,365,974 | 12/1944 | Schreiber      | ----- | 252—400 X |
| 2,530,774 | 11/1950 | Kehe et al.    | ----- | 252—401 X |
| 2,839,563 | 6/1958  | Hechenbleikner |       |           |
| 3,115,465 | 12/1963 | Orloff et al.  |       |           |

DANIEL E. WYMAN, Primary Examiner.

CARL F. DEES, Assistant Examiner.